

# UNITED STATES PATENT OFFICE.

PAUL P. REESE AND SAMUEL S. WALES, OF MUNHALL, PENNSYLVANIA, ASSIGNEES  
TO CARNEGIE STEEL COMPANY, OF PITTSBURGH, PENNSYLVANIA, A CORPORA-  
TION OF NEW JERSEY.

## PROCESS OF MAKING STEEL.

1,082,359.

Specification of Letters Patent. Patented Dec. 23, 1913.

No Drawing.

Application filed January 23, 1912. Serial No. 672,970.

To all whom it may concern:

Be it known that we, PAUL P. REESE and SAMUEL S. WALES, both citizens of the United States, residing at Munhall, in the county of Allegheny and State of Pennsylvania, have invented a new and useful Process of Making Steel, of which the following is a specification.

Our invention relates to the manufacture of open hearth steel of all grades in which the cost of making the steel is not necessarily the governing factor, and while not restricted to such uses, more particularly relates to the manufacture of high grade special steels and alloy steels, and especially those employed in making armor plates, protective deck plates, and like materials.

One object of our invention is to provide an improved process of making steel whereby the temperature and composition of the bath are regulated and the interval of time required in making or completing the heats of steel is varied to the end that the changes in temperature and composition are at all times under the control of the melter and the desired composition is obtained at the time the required pouring temperature of the bath is attained.

A further object of this invention is to provide a novel process of making steel whereby the rate or speed at which the carbon is removed or lessened is regulated and controlled and the too rapid elimination of carbon is prevented, the necessity of "pigging back" the heats is avoided and overcome and the time required in making the steel is lessened or increased as desired.

Another object of our invention is to provide an improved process of making alloy steel by the use of which the necessity of carbon additions other than the amount contained in the final addition of manganese, chrome, or other alloy added at the completion of the heats is avoided and rendered unnecessary.

In carrying out the steps of our improved process, charges, preferably having 40 per cent. iron as a minimum, are put into the furnace in the usual manner. No ore, mill scale or oxid is used in making up the charge, and iron is not employed later in "pigging back" the heats.

After the charge has been completely melt-

ed, (which is preferably effected as rapidly as possible) and the lime has risen to form the slag, an analysis is made and the carbon content of the bath determined. This carbon content will vary largely and should ordinarily be above .75 per cent. An ore addition is then made to the bath of an amount approximating .01 of 1 per cent. of ore for each point of carbon to be removed. Should, after the ore has been thoroughly worked into the bath, the carbon remain at the same or a higher point, a further addition of ore is made at the rate of approximately one-half the amount of the first addition per point of carbon, and the carbon is lessened to approximately .35 to .45 per cent. Additions of ore are not made after the carbon is lessened to about .65 per cent.

When the successive carbon determinations, which are taken at frequent intervals, show the carbon content of the bath to be lessened to about .40 per cent., additions of manganese are made to the bath, the amount of these additions being equal to about .2 of 1 per cent. of manganese or at the rate of about two pounds of 80 per cent. ferro manganese to each one thousand pounds of metallic charge (calculated). Preferably, four such additions are made, in amounts equal to .2 of 1 per cent. at separated intervals after the carbon has been reduced to between .35 and .45 per cent., or a total of .8 per cent. in all. In this way further dropping or elimination of the carbon is retarded, and the removal of the last few points of carbon is caused to extend over a considerable time interval just prior to the tapping operation.

Instead of making the last one or two manganese additions in amounts of .2 of 1 per cent., these amounts may be split up into separately added quantities of .1 of 1 per cent. each.

The additions of manganese are made from time to time so as to preferably prevent the heat of steel being finished when the carbon content is dropping faster than at a rate of one point (.01 per cent.) carbon in a time interval of three minutes.

As it is desired to tap the heats of steel when the desired carbon content is reached, (the amount of carbon added by the additions of ferro alloys being taken into con-

sideration in calculating the charge), the furnace is tapped in the usual way, recarburing in the ladle then being unnecessary, and in making alloy steels, the alloying metals are added as are desired, being added in the usual manner, either in the furnace or in the ladle.

The residual manganese will ordinarily provide the desired amount of manganese in the finished steel. Manganese may be added in the ladle or at the time of tapping when found necessary or desirable. Should it become necessary to hold a heat of steel after being ready to tap, further additions of manganese are made from time to time, the quantity added and the number of additions made depending upon the time interval elapsing between the time the heat reaches the tapping temperature in readiness to tap and the time of tapping.

The process of making high carbon steels is substantially the same as hereinbefore described, the charge being calculated to give a melting point sufficiently high to avoid the necessity of carbon additions other than the amount obtained from the carbon contained in the final addition of manganese, the chrome, or other alloying metal.

In making ordinary steel, the above described steps will be carried out, the additions of manganese being regulated so as to bring the carbon content to the desired point about the time the temperature of the bath reaches the right point for tapping in the manner before described.

The advantages of our invention will be apparent to those skilled in the art. By the use of ferro manganese during the refining of the metal in the furnace, the reduction or elimination of carbon in the bath is at all times under the control of the melter and the making of heats in which the carbon falls below the desired content and requires carburizing is prevented, while the making of heats which are at a proper tapping temperature before the carbon has been reduced to the desired point is avoided.

The use of successive additions of manganese in the bath results in a more thorough and complete removal of sulfur.

The use of ore, cinder or other iron oxide in forming the charge is rendered unnecessary, and the necessity of using coal is overcome.

Variations in the steps of our process may be made without departing from our invention as defined in the claims. The number of additions of manganese may be increased or decreased, and a change in the amount of manganese in each addition may or may not be made as desired, and the amounts of manganese added will vary with steels of different compositions.

We claim:

1. The process of making steel consisting in melting the metallic charge, making additions of ore to the bath to remove carbon therefrom, and then making additions of manganese thereto to check and control the further removal of carbon. 65

2. The process of making steel consisting in melting a charge of scrap steel and iron in which the percentage of steel predominates, making additions of ore to the bath to remove carbon therefrom, and then making additions of manganese thereto to check and control the further removal of carbon. 70 75

3. The process of making steel consisting in melting a charge of scrap steel and iron, making additions of ore to the bath to remove carbon therefrom, and then making successive additions of manganese thereto to thereby check and control the further removal of carbon. 80

4. The process of making steel consisting in rapidly melting a charge of scrap steel and iron in which the percentage of steel predominates, making additions of ore to remove carbon and other metalloids in the charge, and then checking further removal 90 of carbon therefrom by the addition of successively added quantities of manganese. 85

5. The process of making steel consisting in melting a charge of scrap steel and iron in which the percentage of steel predominates, making additions of ore to remove carbon and other metalloids therefrom, and then preventing further removal of carbon by the addition of manganese thereto and tapping the steel when the tapping point is 100 reached. 95

6. The process of making steel consisting in rapidly melting a charge of scrap steel and iron in which the percentage of steel predominates, making additions of ore to remove carbon and other metalloids therefrom, then retarding further removal of carbon by additions of successively added quantities of manganese while bringing the bath to the tapping temperature and then 110 tapping. 105

7. The process of making steel consisting in melting the metallic charge, making additions of ore to rapidly remove a portion of the carbon, then adding manganese in 115 separate successive quantities to retard and prevent further removal of carbon and then tapping the steel when the tapping point is reached, the manganese being added in separate quantities to thereby first retard and then for a short time interval prior to tapping the steel substantially prevent further removal of carbon therefrom. 120

8. The process of making steel consisting in making additions of ore to the molten 125 charge of metal to rapidly remove a portion

of the carbon, then adding manganese to retard and prevent further removal of carbon and then tapping the steel when the tapping point is reached, the manganese being  
5 added in separate quantities to thereby substantially prevent further removal of carbon for a short time interval prior to tapping the steel.

In testimony whereof, we have hereunto set our hands.

PAUL P. REESE.  
SAMUEL S. WALES.

Witnesses:

GEO. B. BLEMING,  
R. D. LITTLE.